

3,184,305  
TITANIUM BASE ALLOYS

Sidney W. Poole and John Savas, Canton, Ohio, assignors to Republic Steel Corporation, Cleveland, Ohio, a corporation of New Jersey  
No Drawing. Filed Oct. 10, 1961, Ser. No. 144,070  
5 Claims. (Cl. 75—175.5)

This invention relates to titanium base alloys. More particularly, this invention relates to titanium base alloys having improved physical and mechanical properties. Still more particularly, this invention relates to titanium base alloys having excellent forgeability, good rollability, low yield in the solution treated condition, and other desirable physical properties. In addition, the alloys of this invention have low solution treating temperatures (1500° F.—1575° F.) which vary in this range depending on section size. The alloys, moreover, are capable of solution treatment by air cooling from these desired low solution annealing temperatures. This is particularly advantageous from a production heat treating standpoint as the use of water quenching techniques during solution treating results in warpage of the materials being so treated. In accordance with one embodiment, this invention is further directed to titanium base alloys having excellent high temperature properties such as improved high temperature tensile and creep properties.

Titanium metal, because of its relatively low density and special high strength and high temperature properties, has been proposed for many uses and in alloys wherein satisfactory performance under high temperature conditions is an important or governing factor. Unfortunately, however, for certain special uses titanium metal and titanium base alloys have not been completely satisfactory. For example, high temperature performance, high temperature tensile strength and creep properties of titanium base alloys available heretofore have been less than desirable.

Accordingly, it is an object of this invention to provide improved titanium base alloys.

It is another object of this invention to provide a titanium base alloy having improved high temperature properties.

Still another object of this invention is to provide titanium base alloys having improved high temperature stress-stability properties.

How these and other objects of this invention are accomplished will become apparent in light of the accompanying disclosure.

A titanium base alloy in accordance with this invention consists essentially of about 7.5—8.5% by weight aluminum, about 9.5—10.5% by weight vanadium, the balance being titanium. The titanium making up the balance of the alloy is substantially pure titanium, such as commercial grade purity titanium, comprising only a very minor amount of incidental impurities. These incidental impurities in the aggregate usually do not amount to more than about 0.3% by weight of the alloy composition and usually include oxygen, normally in an amount not greater than about 0.1%, nitrogen, normally in an amount not greater than about 0.05%, and carbon, normally in an amount not greater than about 0.05%. Hydrogen is also sometimes found as an impurity, normally in an amount not greater than about 0.01%.

Although a titanium base alloy in accordance with this invention, such as an alloy containing 8% by weight aluminum and 10% by weight vanadium, the balance being titanium, shows excellent room temperature properties and stability characteristics, as well as satisfactory short time high temperature properties and satisfactory elevated temperature stress-rupture strengths, in accordance with one embodiment and feature of this invention the elevated temperature properties of the alloy are improved by incorporating therein very minor amounts of silicon or zirconium or both silicon and zirconium. Usually, the amount of either one of these high temperature improving alloying elements, silicon or zirconium, present in any alloy is not greater than about 0.8% by weight.

The following examples are illustrative of the practice of this invention:

## EXAMPLE NO. 1

A titanium base alloy melt having the composition 8.0% by weight aluminum, 10.2% by weight vanadium and 0.53% by weight silicon and containing 0.10% oxygen as an incidental impurity was prepared, forged to 1" round from a temperature of 1900° F. in one heating, and rolled to a  $\frac{5}{8}$ " rod at 1575° F. The thus-prepared  $\frac{5}{8}$ " rod stock was then subjected to various heat treating conditions and the mechanical properties of the heat treated bar stock determined at various temperatures. The results of these tests are set forth in accompanying Table I:

Table I

MECHANICAL PROPERTIES OF  $\frac{5}{8}$ " ROD STOCK AT VARIOUS TEMPERATURES AND IN VARIOUS HEAT TREATED CONDITIONS

| Test temp., °F. | Y.S. (k.s.i.),<br>.2% offset | T.S. (k.s.i.) | R.A.,<br>percent | Elong.,<br>percent in 1" | Heat treatment                               |
|-----------------|------------------------------|---------------|------------------|--------------------------|----------------------------------------------|
| RT              | 179                          | 192           | 34               | 10                       | Ann., 1250° F., A.C.                         |
| 700             | 144                          | 159           | 50               | 13                       | Ann., 1250° F., A.C.                         |
| 1000            | 54                           | 126           | 76               | 30                       | Ann., 1250° F., A.C.                         |
| RT              | 207                          | 217           | 33               | 8                        | S.T., 1475° F., W.Q.; aged, 1000° F., 4 hrs. |
| 800             | 156                          | 176           | 57               | 14                       | S.T., 1475° F., W.Q.; aged, 1000° F., 4 hrs. |
| 800             | 160                          | 173           | 59               | 16                       | S.T., 1475° F., W.Q.; aged, 1000° F., 4 hrs. |
| 1000            | 105                          | 145           | 79               | 29                       | S.T., 1475° F., W.Q.; aged, 1000° F., 4 hrs. |
| RT              | 218                          | 229           | 13               | 4                        | S.T., 1500° F., W.Q.; aged, 1000° F., 4 hrs. |
| 800             | 166                          | 184           | 49               | 13                       | S.T., 1500° F., W.Q.; aged, 1000° F., 4 hrs. |
| 1000            | 97                           | 153           | 80               | 27                       | S.T., 1500° F., W.Q.; aged, 1000° F., 4 hrs. |
| RT              | 210                          | 220           | 29               | 8                        | 1575° F., A.C.; aged, 1000° F., 4 hrs.       |
| 800             | 151                          | 180           | 51               | 14                       | 1575° F., A.C.; aged 1000° F., 4 hrs.        |
| 1000            | 87                           | 152           | 76               | 25                       | 1575° F., A.C.; aged 1000° F., 4 hrs.        |

RT—room temperature.  
A.C.—air cooled.  
W.Q.—water quenched.

S.T.—solution treated.  
Ann.—annealed.

3  
The data set forth in Table I illustrates the exceptionally high mechanical properties obtained by this alloy both at room temperature and at 800° F.

The mechanical properties of this alloy at a temperature of 800° F. are also set forth in Table II together with the properties of other comparable titanium base alloys and a 17-7 PH stainless steel tested at this temperature.

4  
The test results set forth in Table III, like those set forth in Table II, clearly illustrate the superior high temperature properties of a titanium base alloy prepared in accordance with this invention.

#### EXAMPLE NO. 2

Another melt of titanium base alloy in accordance with this invention analyzing 8.65% by weight aluminum,

5  
*Table II*  
HOT TENSILE PROPERTIES OF VARIOUS ALLOYS AT 800° F.

| Alloy                     | Y.S. (k.s.i.),<br>.2% offset | T.S. (k.s.i.) | R.A.,<br>percent | Elong.,<br>percent in 1" | Heat treatment                                |
|---------------------------|------------------------------|---------------|------------------|--------------------------|-----------------------------------------------|
| 8 Al-10.2 V-5 Si          | 156                          | 176           | 57               | 14                       | S.T., 1475° F., W.Q.; aged, 1000° F., 4 hrs.  |
|                           | 160                          | 173           | 59               | 16                       | S.T., 1475° F., W.Q.; aged, 1000° F., 4 hrs.  |
|                           | 166                          | 184           | 49               | 13                       | S.T., 1500° F., W.Q.; aged, 1000° F., 4 hrs.  |
| 5 Al-2.75 Cr-1.25 Fe      | 151                          | 180           | 51               | 14                       | 1575° F., A.C.; aged 1000° F., 4 hrs.         |
|                           | 109                          | 133           | 64               | 15                       | S.T., 1450° F., W.Q.; aged, 900° F., 5 hrs.   |
| 5 Al-1.5 Fe-1.4 Cr-1.2 Mo | 112                          | 133           | 73               | 17                       | S.T., 1600° F., W.Q.; aged, 1000° F., 24 hrs. |
| 6 Al-4 V                  | 85                           | 105           | 57               | 18                       | S.T., 1550° F., W.Q.; aged, 900° F., 24 hrs.  |
| 16 V-2.5 Al               | 120                          | 132           | -----            | 7                        | S.T., 1370° F., W.Q.; aged, 900° F., 24 hrs.  |
| 4 Al-4 Mn                 | 90                           | 110           | 48               | 15                       | S.T., 1450° F., W.Q.; aged, 900° F., 6 hrs.   |
| 2 Fe-2 Cr-2 Mo            | 84                           | 120           | 89               | 26                       | S.T., 1480° F., W.Q.; aged, 900° F., 24 hrs.  |
| 8 Al-2 Cb-1 Ta            | 70                           | 92            | 53               | 28                       | Milled annealed alpha alloy.                  |
| 5 Al-2.5 Sn               | 60                           | 77            | 45               | 17                       | Do.                                           |
| 17-7 PH stainless steel   | 152                          | 182           | -----            | -----                    | Heat treated; aged, 900° F.                   |

The test data set forth in Table II illustrates the exceptional high temperature properties of a titanium base alloy prepared in accordance with this invention. Further, the test properties of this alloy carried out at a temperature of 1000° F. are set forth in Table III and compared with the tensile properties of other titanium base alloys and a 17-7 PH stainless steel tested at this temperature.

35  
10.34% by weight vanadium and with the balance titanium, and containing 0.09% by weight oxygen as an incidental impurity, was forged to 1" round from 1900° F. and rolled to  $\frac{5}{8}$ " bar at 1575° F. The mechanical properties of samples of the resulting bar stock were then tested at various temperatures and in various heat treated

*Table III*  
HOT TENSILE PROPERTIES OF VARIOUS ALLOYS AT 1000° F.

| Alloy                     | Y.S. (k.s.i.),<br>.2% offset | T.S. (k.s.i.) | R.A.,<br>percent | Elong., | Heat treatment                                |
|---------------------------|------------------------------|---------------|------------------|---------|-----------------------------------------------|
| 8 Al-10.2 V-5 Si          | 105                          | 145           | 79               | 29      | S.T., 1475° F., W.Q.; Aged, 1000° F., 4 hrs.  |
|                           | 97                           | 153           | 80               | 27      | S.T., 1500° F., W.Q.; aged, 1000° F., 4 hrs.  |
|                           | 87                           | 152           | 76               | 25      | 1575° F., A.C.; aged, 1000° F., 4 hrs.        |
| 5 Al-2.75 Cr-1.25 Fe      | 79                           | 92            | 82               | 36      | S.T., 1450° F., W.Q.; aged, 900° F., 5 hrs.   |
|                           | 79                           | 92            | 83               | 40      | S.T., 1600° F., W.Q.; aged, 1000° F., 24 hrs. |
| 5 Al-1.5 Fe-1.4 Cr-1.2 Mo | 78                           | 112           | 83               | 30      | S.T., 1550° F., W.Q.; aged, 900° F., 24 hrs.  |
|                           | 70                           | 81            | 71               | 31      | S.T., 1750° F., W.Q.; aged, 900° F., 2 hrs.   |
| 6 Al-4 V                  | 73                           | 94            | 86               | 21      | S.T., 1450° F., W.Q.; aged, 900° F., 6 hrs.   |
|                           | 82                           | 97            | 55               | 21      | S.T., 1480° F., W.Q.; aged, 900° F., 24 hrs.  |
| 2 Fe-2 Cr-2 Mo            | 25                           | 53            | 98               | 93      | Milled annealed alpha alloy.                  |
| 8 Al-2 Cb-1 Ta            | 66                           | 79            | 55               | 33      | Do.                                           |
| 5 Al-2.5 Sn               | 54                           | 67            | 47               | 18      | Heat treated; aged 900° F.                    |
| 17-7 PH stainless steel   | 105                          | 130           | -----            | -----   | -----                                         |

conditions. The results of these tests are set forth in accompanying Table IV:

*Table IV*  
MECHANICAL PROPERTIES OF  $\frac{5}{8}$ " BAR STOCK AT VARIOUS TEMPERATURES AND IN VARIOUS HEAT TREATED CONDITIONS

| Sample No. | Test temp. | Y.S. (k.s.i.),<br>.2% offset | T.S. (k.s.i.) | R.A.,<br>percent | Elong.,<br>percent in 1" | Heat Treatment                                    |
|------------|------------|------------------------------|---------------|------------------|--------------------------|---------------------------------------------------|
| 4-13       | R.T.       | 169.2                        | 183.6         | 28               | 8                        | As Rolled (1575° F.).                             |
| 4-1        | R.T.       | 170.3                        | 182.7         | 29               | 9                        | Annealed, 1250° F., A.C.                          |
| 4-2        | R.T.       | 156.2                        | 180.9         | 26               | 8                        | Annealed, 1575° F., A.C.                          |
| 4-3        | R.T.       | 207.2                        | 221.7         | 27               | 8                        | Sol. ann., 1575° F., A.C., Aged, 900° F., 10 hrs. |
| 4-6        | R.T.       | 197.8                        | 210.4         | 31               | 8                        | Sol. ann., 1575° F., A.C., aged, 1000° F., 8 hrs. |
| 4-4        | 800° F.    | 149.8                        | 173.3         | 63               | 15                       | Sol. ann., 1575° F., A.C., aged, 900° F., 10 hrs. |

Table IV—Continued

CREEP TESTS—SUBJECTED TO 65,000 P.S.I. FOR 100 HRS. AT 800° F.—PULLED AT ROOM TEMPERATURE AFTER CREEP EXPOSURE\*

| Sample No. | Test temp.      | Y.S. (k.s.i.),<br>.2% offset | T.S. (k.s.i.) | R.A.,<br>percent | Elong.,<br>percent in 1" | Heat Treatment                                       |
|------------|-----------------|------------------------------|---------------|------------------|--------------------------|------------------------------------------------------|
| 4-5-----   | .74% creep----- | 203.0                        | 224.2         | 21               | 7                        | Sol. ann., 1575° F., A.C., aged,<br>900° F., 10 hrs. |
| 4-7-----   | .82% creep----- | 197.0                        | 214.6         | 24               | 7.5                      | Sol. ann., 1575° F., A.C., aged,<br>1000° F., 8 hrs. |
| 4-8-----   | .83% creep----- | 193.5                        | 209.9         | 30               | 9.5                      | Sol. ann., 1575° F., A.C., aged,<br>1100° F., 4 hrs. |

\* The specimens were pulled with discoloration on the gage length from previous creep exposure.

## EXAMPLE NO. 3

Another melt of titanium base alloy in accordance

conditions. The results of these tests are set forth in accompanying Table V.

Table V

MECHANICAL PROPERTIES OF  $\frac{5}{8}$ " BAR STOCK AT VARIOUS TEMPERATURES AND IN VARIOUS HEAT TREATED CONDITIONS

| Sample No. | Test temp.   | Y.S. (k.s.i.),<br>.2% offset | T.S. (k.s.i.) | R.A.,<br>percent | Elong.,<br>percent in 1" | Heat Treatment                                       |
|------------|--------------|------------------------------|---------------|------------------|--------------------------|------------------------------------------------------|
| 3-13-----  | R.T.-----    | 172.0                        | 188.6         | 21               | 6                        | As rolled (1575° F.).                                |
| 3-1-----   | R.T.-----    | 172.5                        | 185.8         | 16               | 6                        | Annealed, 1250° F., A.C.                             |
| 3-2-----   | R.T.-----    | 161.3                        | 180.6         | 14               | 6                        | Annealed, 1575° F., A.C.                             |
| 3-9-----   | R.T.-----    | 201.8                        | 212.7         | 9                | 4                        | Sol. ann., 1550° F., A.C., aged,<br>1000° F., 8 hrs. |
| 3-10-----  | R.T.-----    | 196.4                        | 206.5         | 9                | 4                        | Sol. ann., 1550° F., A.C., aged,<br>1050° F., 4 hrs. |
| 3-3-----   | R.T.-----    | 225.5                        | 241.8         | 17               | 4                        | Sol. ann., 1575° F., A.C., aged,<br>900° F., 10 hrs. |
| 3-6-----   | R.T.-----    | 211.5                        | 224.1         | 14               | 5                        | Sol. ann., 1575° F., A.C.; aged,<br>1000° F., 8 hrs. |
| 3-4-----   | 800° F.----- | 164.2                        | 193.4         | 43               | 11                       | Sol. ann., 1575° F., A.C., aged,<br>900° F., 10 hrs. |

CREEP TESTS—SUBJECTED TO 65,000 P.S.I. FOR 100 HRS. AT 800° F.—PULLED AT ROOM TEMPERATURE AFTER CREEP EXPOSURE\*

|          |                 |       |       |   |     |                                                      |
|----------|-----------------|-------|-------|---|-----|------------------------------------------------------|
| 3-5----- | .20% creep----- | 216.2 | 240.4 | 6 | 3   | Sol. ann., 1750° F., A.C., aged,<br>900° F., 10 hrs. |
| 3-7----- | .04% creep----- | 215.2 | 232.8 | 7 | 4   | Sol. ann., 1575° F., A.C.; aged,<br>1000° F., 8 hrs. |
| 3-8----- | .44% creep----- | 201.6 | 216.6 | 4 | 3.5 | Sol. ann., 1575° F., A.C., Aged<br>1100° F., 4 hrs.  |

\* The specimens were pulled with discoloration on the gage length from previous creep exposure.

with this invention analyzing 8.51% of aluminum, 10.20% vanadium, 0.74% zirconium, 0.59% silicon, the balance being titanium, together with 0.08% by weight oxygen as an incidental impurity, was prepared, forged to 1" round at 1900° F. and rolled to  $\frac{5}{8}$ " bar at 1575° F. Samples of this bar stock were then subjected to various tests at various temperatures and in various heat treated

45

Samples of  $\frac{5}{8}$ " bar stock of various titanium base alloys having a composition in accordance with this invention were tested at various temperatures and in various heat treated conditions. The results of these tests are set forth in accompanying Table VI:

Table VI

MECHANICAL PROPERTIES OF  $\frac{5}{8}$ " BAR STOCK AT VARIOUS MODIFICATIONS OF Ti-8 Al-10 V ALLOY COMPOSITION AS RELATED TO HEAT TREATMENT AND TEST TEMPERATURE

[Tensile properties]

| Actual analysis |      |    |    | Test temp.   | Y.S. (k.s.i.),<br>.2% offset | T.S. (k.s.i.) | R.A.,<br>percent | Elong,<br>percent | Heat treatment                            |
|-----------------|------|----|----|--------------|------------------------------|---------------|------------------|-------------------|-------------------------------------------|
| Al              | V    | Zr | Si |              |                              |               |                  |                   |                                           |
| 7.8             | 10.0 |    |    | R.T.-----    | 168.2                        | 181.0         | 32               | 11                | Ann., 1250° F., A.C.                      |
|                 |      |    |    | R.T.-----    | 202.6                        | 218.9         | 36               | 8                 | 1575° F., A.C.; aged,<br>900° F., 10 hrs. |
|                 |      |    |    | R.T.-----    | 194.6                        | 209.9         | 36               | 10                | 1575° F., A.C.; aged,<br>1000° F., 8 hrs. |
|                 |      |    |    | 800° F.----- | 156.0                        | 172.1         | 63               | 14                | 1575° F., A.C.; aged,<br>900° F., 10 hrs. |
|                 |      |    |    | 800° F.----- | 144.2                        | 164.7         | 62               | 15.5              | 1575° F., A.C.; aged,<br>1000° F., 8 hrs. |
| 8.6             | 10.3 |    |    | R.T.-----    | 170.3                        | 182.7         | 29               | 9                 | Ann., 1250° F., A.C.                      |
|                 |      |    |    | R.T.-----    | 207.2                        | 221.7         | 27               | 8                 | 1575° F., A.C.; aged,<br>900° F., 10 hrs. |
|                 |      |    |    | R.T.-----    | 197.8                        | 210.4         | 31               | 8                 | 1575° F., A.C.; aged,<br>1000° F., 8 hrs. |
|                 |      |    |    | 800° F.----- | 149.8                        | 173.3         | 63               | 15                | 1575° F., A.C.; aged,<br>900° F., 10 hrs. |
| 8.0             | 10.5 |    | .4 | R.T.-----    | 178.3                        | 193.8         | 29               | 9                 | Ann., 1250° F., A.C.                      |
|                 |      |    |    | R.T.-----    | 200.2                        | 212.2         | 19               | 7                 | 1575° F., A.C.; aged,<br>1000° F., 8 hrs. |
|                 |      |    |    | 800° F.----- | 144.7                        | 166.0         | 54               | 16                | 1575° F., A.C.; aged,<br>1000° F., 6 hrs. |
| 8.0             | 10.2 |    | .5 | R.T.-----    | 179.0                        | 192.0         | 34               | 10                | Ann., 1250° F., A.C.                      |
|                 |      |    |    | R.T.-----    | 210.0                        | 220.0         | 29               | 8                 | 1575° F., A.C.; aged,<br>1000° F., 4 hrs. |

Table VI—Continued

MECHANICAL PROPERTIES OF  $\frac{1}{4}$ " BAR STOCK AT VARIOUS MODIFICATIONS OF Ti-8 Al-10 V ALLOY  
COMPOSITION AS RELATED TO HEAT TREATMENT AND TEST TEMPERATURE  
[Tensile properties]

| Actual analysis |      |    |    | Test temp. | Y.S. (k.s.i.),<br>2% offset | T.S. (k.s.i.) | R.A.,<br>percent | Elong,<br>percent | Heat treatment                            |
|-----------------|------|----|----|------------|-----------------------------|---------------|------------------|-------------------|-------------------------------------------|
| Al              | V    | Zr | Si |            |                             |               |                  |                   |                                           |
| 8.0             | 9.8  | .7 |    | 800° F.    | 151.0                       | 180.0         | 51               | 14                | 1575° F., A.C.; aged,<br>1000° F., 4 hrs. |
|                 |      |    |    | 1000° F.   | 87.0                        | 152.0         | 76               | 25                | 1575° F., A.C.; aged,<br>1000° F., 4 hrs. |
|                 |      |    |    | R.T.       | 176.5                       | 192.5         | 27               | 10                | Ann., 1250° F., A.C.                      |
|                 |      |    |    | R.T.       | 213.6                       | 229.4         | 15               | 5                 | 1575° F., A.C.; aged,<br>900° F., 10 hrs. |
|                 |      |    |    | R.T.       | 197.2                       | 213.0         | 15               | 6.5               | 1575° F., A.C.; aged,<br>1000° F., 8 hrs. |
|                 |      |    |    | 800° F.    | 164.5                       | 186.1         | 43               | 10                | 1575° F., A.C.; aged,<br>900° F., 10 hrs. |
| 7.8             | 9.5  | .5 |    | 800° F.    | 151.2                       | 171.8         | 43               | 12                | 1575° F., A.C.; aged,<br>1000° F., 8 hrs. |
|                 |      |    |    | R.T.       | 159.7                       | 174.1         | 46               | 12                | Ann., 1250° F., A.C.                      |
|                 |      |    |    | R.T.       | 196.4                       | 216.3         | 34               | 8                 | 1575° F., A.C.; aged,<br>900° F., 10 hrs. |
|                 |      |    |    | 800° F.    | 138.0                       | 166.4         | 63               | 14                | 900° F., 10 hrs.                          |
| 8.0             | 10.1 | .6 | .5 | R.T.       | 176.3                       | 190.4         | 25               | 7                 | Ann., 1250° F., A.C.                      |
|                 |      |    |    | R.T.       | 202.8                       | 214.6         | 26               | 8                 | 1575° F., A.C.; aged,<br>1000° F., 6 hrs. |
|                 |      |    |    | 800° F.    | 154.6                       | 175.9         | 31               | 11                | 1575° F., A.C.; aged,<br>1000° F., 6 hrs. |
| 8.5             | 10.2 | .7 | .6 | R.T.       | 172.5                       | 185.8         | 16               | 6                 | Ann., 1250° F., A.C.                      |
|                 |      |    |    | R.T.       | 222.5                       | 241.8         | 17               | 4                 | 1575° F., A.C.; aged,<br>900° F., 10 hrs. |
|                 |      |    |    | R.T.       | 211.5                       | 224.1         | 14               | 5                 | 1575° F., A.C.; aged,<br>1000° F., 8 hrs. |
|                 |      |    |    | 800° F.    | 164.2                       | 193.4         | 43               | 11                | 1575° F., A.C.; aged,<br>900° F., 10 hrs. |

Additional tests were carried out to determine the creep and stress stability properties at 800° F. of the various alloys having compositions in accordance with this invention. The results of these tests are set forth in accompanying Table VII.

35

An analysis of the data set forth in Tables VI and VII, and in Tables IV and V indicates that a titanium base alloy having a composition in the range 7.5–8.5% by weight aluminium, 9.5–10.5% by weight vanadium, the balance being titanium, particularly a titanium base alloy

TABLE VII

CREEP AND CREEP-STABILITY PROPERTIES OF  $\frac{1}{4}$ " BAR STOCK AT VARIOUS MODIFICATIONS OF THE Ti-8 Al-10 V ALLOY COMPOSITION

[Creep tests—Subjected to 65,000 p.s.i. for 100 hrs. at 800° F. Pulled at room temperature after creep exposure]

| Actual analysis |      |    |    | Creep      | Y.S. (k.s.i.),<br>2% offset | T.S. (k.s.i.) | R.A.,<br>percent | Elong,<br>percent | Heat treatment                                       |
|-----------------|------|----|----|------------|-----------------------------|---------------|------------------|-------------------|------------------------------------------------------|
| Al              | V    | Zr | Si |            |                             |               |                  |                   |                                                      |
| 7.8             | 10.0 |    |    | 1.44%----- | 197.5                       | 220.2         | 35               | 9                 | Sol. ann., 1575° F., A.C.;<br>aged, 900° F., 10 hrs. |
|                 |      |    |    | .74%-----  | 193.9                       | 216.0         | 25               | 9                 | Sol. ann., 1575° F., A.C.;<br>aged, 1000° F., 8 hrs. |
|                 |      |    |    | .67%-----  | 190.2                       | 209.0         | 32               | 10                | Sol. ann., 1575° F., A.C.;<br>aged, 1050° F., 4 hrs. |
| 8.6             | 10.3 |    |    | .74%-----  | 203.0                       | 224.2         | 21               | 7                 | Sol. ann., 1575° F., A.C.;<br>aged, 900° F., 10 hrs. |
|                 |      |    |    | .82%-----  | 197.0                       | 214.6         | 24               | 7.5               | Sol. ann., 1575° F., A.C.;<br>aged, 1000° F., 8 hrs. |
|                 |      |    |    | .83%-----  | 193.5                       | 209.9         | 30               | 9.5               | Sol. ann., 1575° F., A.C.;<br>aged, 1100° F., 4 hrs. |
| 8.0             | 10.5 | .4 |    | 1.0%-----  | 194.3                       | 214.7         | 23               | 8                 | Sol. ann., 1575° F., A.C.;<br>aged, 1000° F., 6 hrs. |
|                 |      |    |    | 1.0%-----  | 197.3                       | 215.9         | 27               | 9                 | Sol. ann., 1575° F., A.C.;<br>aged, 1050° F., 4 hrs. |
| 8.0             | 10.2 |    | .5 | .91%-----  | 207.7                       | 224.8         | 30               | 8                 | S.T., 1475° F., W.Q.;<br>aged, 1000° F., 4 hrs.      |
| 8.0             | 9.8  |    | .7 | .63%-----  | 210.3                       | 232.7         | 21               | 7                 | Sol. ann., 1575° F., A.C.;<br>aged, 900° F., 10 hrs. |
|                 |      |    |    | .82%-----  | 198.9                       | 217.8         | 15               | 6.5               | Sol. ann., 1575° F., A.C.;<br>aged, 1000° F., 8 hrs. |
|                 |      |    |    | .86%-----  | 199.2                       | 216.4         | 26               | 8                 | Sol. ann., 1575° F., A.C.;<br>aged, 1050° F., 4 hrs. |
| 7.3             | 9.5  | .5 |    | .55%-----  | 191.2                       | 218.8         | 30               | 8                 | Sol. ann., 1575° F., A.C.;<br>aged, 900° F., 10 hrs. |
|                 |      |    |    | .78%-----  | 190.8                       | 209.6         | 33               | 10                | Sol. ann., 1575° F., A.C.;<br>aged, 1000° F., 8 hrs. |
| 8.0             | 10.1 | .6 | .5 | .2%-----   | 214.6                       | 234.8         | 16               | 4.5               | Sol. ann., 1575° F., A.C.;<br>aged, 1000° F., 6 hrs. |
|                 |      |    |    | .4%-----   | 211.5                       | 227.0         | 24               | 6.5               | Sol. ann., 1575° F., A.C.;<br>aged, 1050° F., 4 hrs. |
| 8.5             | 10.2 | .7 | .6 | .20%-----  | 216.2                       | 240.4         | 6                | 3                 | Sol. ann., 1575° F., A.C.;<br>aged, 900° F., 10 hrs. |
|                 |      |    |    | .04%-----  | 215.2                       | 232.8         | 7                | 4                 | Sol. ann., 1575° F., A.C.;<br>aged, 1000° F., 8 hrs. |
|                 |      |    |    | .44%-----  | 201.4                       | 216.6         | 4                | 3.5               | Sol. ann., 1575° F., A.C.;<br>aged, 1100° F., 4 hrs. |

containing about 8% by weight aluminum and about 10% by weight vanadium, exhibits excellent room temperature tensile properties with good ductility. These test data also indicate that the alloy compositions of this invention have excellent high temperature tensile properties, particularly at about 800° F. The test data also indicate that the addition of not more than about 0.7% silicon improves the annealed properties of the base alloy without a loss in tensile ductility. The test data clearly set forth that this amount of silicon also improves the high temperature tensile properties of the alloy.

The test data also indicate that up to about 0.7% silicon can be present in the base alloy without a serious drop in tensile ductility and that the addition of not more than 0.6% zirconium together with not more than 0.5% silicon to the base alloy further improves the high temperature tensile properties of the alloy at 800° F. The addition of zirconium further improves the creep resistance of the base alloy and modified only by the addition of silicon. Zirconium additions to the base alloy, however, in excess of 0.6% in conjunction with silicon additions in excess of 0.5% appear to be detrimental to the room temperature properties and stability of the particular alloy of this invention. These test data also indicate that for best high temperature tensile properties an aging treatment of about 900° F. for 10 hours is recommended after annealing the alloy at 1575° F. followed by air cooling.

Generally, it has been determined that the titanium base alloys of this invention, such as an alloy having the composition about 8% by weight aluminum, about 10% by weight vanadium, the balance being titanium with incidental impurities, is at least 15% better in tensile properties at room temperature than any commercial bar alloy and at 800° F. this percentage increases. Further, the base alloy of this invention comprising 8% by weight aluminum, 10% by weight vanadium modified with very minor amounts of zirconium and silicon show even greater percentage differences at higher temperatures up to 800° F. Also, on a strength-to-weight basis at 800° F. the zirconium and silicon modified titanium base alloy of this invention is about twice as good as the standard grades of precipitation hardening stainless steels.

In a titanium base alloy sheet product having a composition in accordance with this invention the only commercially available titanium sheet alloy that approaches it is a beta grade alloy containing 13% vanadium, 11% chromium, 3% aluminum, the balance being titanium. The disadvantages of the beta grade titanium alloy, however, are its higher density and longer ageing times required to reach optimum properties. Further, the stability of the beta alloy at a temperature about 600° F. is questionable.

Tables VIII and IX show the superiority in respect to certain physical properties of a titanium base alloy having a composition in accordance with this invention as compared with other titanium alloys.

Table VIII

## BAR PRODUCT

[Ti-8 Al-10 V]

| Test temp. | Y.S. (k.s.i.), 0.2% offset | T.S. (k.s.i.) | R.A., percent | Elong., percent | Heat treatment                         |
|------------|----------------------------|---------------|---------------|-----------------|----------------------------------------|
| R.T.       | 170                        | 180           | 30            | 10              | Ann.                                   |
| R.T.       | 195                        | 210           | 30            | 9               | 1575° F., A.C.; aged, 1000° F., 8 hrs. |
| R.T.       | 205                        | 220           | 30            | 8               | 1575° F., A.C.; aged, 900° F., 10 hrs. |
| 800° F.    | 145                        | 165           | 60            | 15              | 1575° F., A.C.; aged, 1000° F., 8 hrs. |
| 800° F.    | 150                        | 170           | 60            | 14              | 1575° F., A.C.; aged, 900° F., 10 hrs. |

[Ti-7 Al-4 Mo]

|      |     |     |  |    |                                        |
|------|-----|-----|--|----|----------------------------------------|
| R.T. | 150 | 160 |  | 15 | Ann.                                   |
| R.T. | 175 | 190 |  | 12 | 1650° F., W.Q.; aged, 900° F., 16 hrs. |

[Ti-6 Al-4 V]

|         |     |     |    |    |                                       |
|---------|-----|-----|----|----|---------------------------------------|
| R.T.    | 136 | 148 | 43 | 15 | Ann.                                  |
| R.T.    | 145 | 152 | 43 | 15 | 1550° F., 24 hrs.                     |
| R.T.    | 155 | 164 | 43 | 16 | 1750° F., W.Q.; aged, 900° F., 2 hrs. |
| 800° F. | 85  | 98  | 55 | 15 | Ann.                                  |
| 800° F. | 85  | 105 | 57 | 18 | 1550° F., 24 hrs.                     |
| 800° F. | 90  | 115 | 72 | 18 | 1750° F., W.Q.; aged, 900° F., 2 hrs. |

[Ti-4 Al-4 Mn]

|      |     |     |  |    |                                        |
|------|-----|-----|--|----|----------------------------------------|
| R.T. | 133 | 148 |  | 16 | Ann.                                   |
| R.T. | 140 | 162 |  | 9  | 1450° F., W.Q.; aged, 900° F., 24 hrs. |

Table IX  
SHEET PRODUCT  
[Ti-8 Al-10 V]

| Test temp. | Direction | Y.S. (k.s.i.),<br>0.2% offset | T.S.<br>(k.s.i.) | Elong.,<br>percent in 2" | Heat treatment                         |
|------------|-----------|-------------------------------|------------------|--------------------------|----------------------------------------|
| R.T.       | Long      | 193.7                         | 209.8            | 4.5                      | 1500° F., A.C.; aged, 1000° F., 4 hrs. |
| R.T.       | Trans     | 194.8                         | 208.7            | 6.5                      | 1500° F., A.C., aged, 1000° F., 4 hrs. |
| R.T.       | Long      | 202.9                         | 225.4            | 4                        | 1500° F., A.C.; aged, 900° F., 10 hrs. |
| R.T.       | Trans     | 209.6                         | 229.2            | 4.5                      | 1500° F., A.C.; aged, 900° F., 10 hrs. |
| 800° F.    | Long      | 150.7                         | 184.3            | 3.5                      | 1500° F., A.C.; aged, 900° F., 10 hrs. |

[Ti-6 Al-4 V]

|      |  |     |     |    |                                       |
|------|--|-----|-----|----|---------------------------------------|
| R.T. |  | 120 | 135 | 11 | Ann.                                  |
| R.T. |  | 150 | 170 | 7  | 1700° F., W.Q.; aged, 975° F., 8 hrs. |

[Ti-5 Al-2.75 Cr-1.25 Fe]

|      |  |     |     |    |                                       |
|------|--|-----|-----|----|---------------------------------------|
| R.T. |  | 135 | 155 | 14 | Ann.                                  |
| R.T. |  | 165 | 195 | 6  | 1475° F., W.Q.; aged, 900° F., 5 hrs. |

[Ti-3 Al-13 V-11 Cr (beta alloy)]

|         |       |       |       |   |                                        |
|---------|-------|-------|-------|---|----------------------------------------|
| R.T.    | Long  | 165.8 | 176.1 | 4 | 1400° F., A.C.; aged, 850° F., 36 hrs. |
| R.T.    | Trans | 164.5 | 182.3 | 6 | 1400° F., A.C.; aged, 850° F., 36 hrs. |
| R.T.    | Long  | 178.5 | 198.0 | 5 | 1400° F., A.C.; aged, 900° F., 72 hrs. |
| R.T.    | Trans | 185.6 | 203.0 | 3 | 1400° F., A.C.; aged, 900° F., 72 hrs. |
| 800° F. | Long  | 131.8 | 149.6 | 6 | 1400° F., A.C.; aged, 850° F., 36 hrs. |
| 800° F. | Trans | 131.5 | 155.1 | 5 | 1400° F., A.C.; aged, 850° F., 36 hrs. |
| 800° F. | Long  | 141.2 | 167.2 | 5 | 1400° F., A.C., aged, 900° F., 72 hrs. |
| 800° F. | Trans | 146.6 | 170.7 | 7 | 1400° F., A.C.; aged, 900° F., 72 hrs. |

## EXAMPLE NO. 5

A titanium base alloy melt having the composition 7.26% aluminum, 9.48% vanadium, 0.50% zirconium, 0.09% silicon, the balance being titanium with 0.09% 45

this composition and samples of this bar stock were tested at various temperatures and in various heat treated conditions. The results of these tests are set forth in accompanying Table X:

Table X  
MECHANICAL PROPERTIES OF 5/8" BAR STOCK AT VARIOUS TEMPERATURES AND IN VARIOUS HEAT TREATED CONDITIONS

| Sample No. | Test temp. | Y.S. (k.s.i.),<br>2% offset | T.S. (k.s.i.) | R.A.,<br>percent | Elong.,<br>percent in 1" | Heat Treatment                                    |
|------------|------------|-----------------------------|---------------|------------------|--------------------------|---------------------------------------------------|
| 13         | R.T.       | 159.7                       | 174.1         | 46               | 12                       | As rolled (1575° F.).                             |
| 7          | R.T.       | 163.3                       | 176.3         | 40               | 12                       | Annealed, 1250° F., A.C.                          |
| 8          | R.T.       | 148.3                       | 175.3         | 36               | 10                       | Annealed, 1575° F., A.C.                          |
| 1          | R.T.       | 196.4                       | 216.3         | 34               | 8                        | Sol. ann., 1575° F., A.C.; aged, 900° F., 10 hrs. |
| 4          | R.T.       | 190.3                       | 201.8         | 38               | 10                       | Sol. ann., 1575° F., A.C.; aged, 1000° F., 8 hrs. |
| 2          | 800° F.    | 138.0                       | 166.4         | 63               | 14                       | Sol. ann., 1575° F., A.C.; aged, 900° F., 10 hrs. |
| 5          | 800° F.    | 138.5                       | 158.6         | 64               | 15                       | Sol. ann., 1575° F., A.C.; aged, 1000° F., 8 hrs. |

CREEP TESTS—SUBJECTED TO 65,000 P.S.I. FOR 100 HRS. AT 800° F.—PULLED AT ROOM TEMPERATURE AFTER CREEP EXPOSURE\*

|   |            |       |       |    |    |                                                   |
|---|------------|-------|-------|----|----|---------------------------------------------------|
| 3 | .55% creep | 191.2 | 218.8 | 30 | 8  | Sol. ann., 1575° F., A.C.; aged, 900° F., 10 hrs. |
| 6 | .78%       | 190.8 | 209.6 | 33 | 10 | Sol. ann., 1575° F., A.C.; aged, 1000° F., 8 hrs. |

\*Indicates specimens were pulled with discoloration on gage length.

oxygen as an incidental impurity, was prepared to check the creep properties of the zirconium modified alloy. The approximate 0.1% silicon content in the alloy was introduced from the master alloys employed in making up the melt. 5/8 bar stock was fabricated from the alloy having 75 base alloy compositions of this invention, the overall

It is pointed out that because the aluminum content of this particular alloy tested analyzed relatively low about 7.25% by weight aluminum, instead of the usual 8.0% aluminum found in the nominal 8% Al, 10% V, titanium

properties were slightly below the capabilities of the Ti-8Al-10V composition. The creep properties, however, were improved by the zirconium addition but to the degree that the combination of the zirconium and silicon additions, limited to about 0.5% each, improves these properties.

## EXAMPLE NO. 6

The titanium base alloy of Example No. 2, having the composition 8.65% aluminum, 10.34% vanadium, the balance being titanium, together with 0.09% oxygen as an incidental impurity, was further tested to determine the Charpy V-notch impact properties of the nominal alloy of this invention. The  $\frac{5}{8}$ " bar stock was heat treated as shown to correlate the impact properties of the alloy to the tensile properties previously developed. The result of these tests are set forth in accompanying Table XI:

Table XI

| Y.S. (k.s.i.),<br>.2% offset | T.S. (k.s.i.) | R.A.,<br>percent | Elong., per-<br>cent in 1" | Charpy im-<br>pact, ft.-lbs.<br>(-40° F.) | Heat treatment                                                           |
|------------------------------|---------------|------------------|----------------------------|-------------------------------------------|--------------------------------------------------------------------------|
| 170.3                        | 182.7         | 29               | 9                          | 8.5                                       | Annealed 1250° F., A.C.                                                  |
| 207.2                        | 221.7         | 27               | 8                          | 9.5                                       | Sol. ann., 1575° F., A.C.; aged,                                         |
| 197.8                        | 210.4         | 31               | 8                          | 8                                         | 900° F., 10 hrs.<br>Sol. ann., 1575° F., A.C., aged,<br>1000° F., 8 hrs. |

The test data in Table XI show that the Charpy impact properties at  $-40^{\circ}$  F. and at the high tensile levels indicated are very good for these titanium base alloys.

The titanium base alloys having compositions in accordance with this invention may be prepared by any suitable and convenient method, such as melting one or more of the master alloys making up the final alloy composition and adding the other metals thereto in the desired amounts or proportions to yield the desired alloy composition. The alloy is conveniently made by melting an admixture of two or more of master alloys making up the alloy together with sponge titanium. For example, the metal alloy constituents individually in powder, granular or fragment form can be mixed as convenient and formed into a compact mass used as an arc electrode under appropriate conditions to yield an ingot of the finished alloy. The elements making up the composition are thus melted into ingot form. Although a procedure of this type is especially effective and thus is of unusual advantage or convenience, other methods of preparation of the alloys of this invention may be employed having appropriate regard for such matters as operating convenience and the desired type or use of the product.

As will be apparent to those skilled in the art in the light of the foregoing disclosure many modifications, substitutions, or alterations are possible in the practice of this invention without departing from the spirit or scope thereof.

We claim:

1. A titanium base alloy consisting essentially of about 7.5-8.5% aluminum, about 9.5-10.5% vanadium, 0.1-0.5% silicon, about 0.1-0.6% zirconium, the balance being commercial grade purity titanium.

2. A titanium base alloy consisting essentially of about 8% by weight aluminum, 10% by weight vanadium, 0.1-0.6% by weight silicon, the balance being commercial grade purity titanium.

3. A titanium base alloy having a composition in accordance with claim 2 wherein silicon and zirconium are present in substantially equal amounts by weight.

4. A titanium base alloy having a composition in accordance with claim 2 wherein the incidental impurities present in the titanium are not greater than about 0.3% by weight based on said alloy.

5. A titanium base alloy consisting essentially of about 8% by weight aluminum, about 10% by weight vanadium about 0.6% by weight zirconium, about 0.5% by weight silicon, the balance being commercial grade titanium.

## References Cited by the Examiner

## UNITED STATES PATENTS

|           |       |                |       |          |
|-----------|-------|----------------|-------|----------|
| 2,754,204 | 7/56  | Jaffee et al.  | ----- | 75-175.5 |
| 2,754,205 | 7/56  | Jaffee et al.  | ----- | 75-175.5 |
| 2,804,409 | 8/57  | Kessler et al. | ----- | 75-175.5 |
| 2,918,367 | 12/59 | Crossley       | ----- | 75-175.5 |

## FOREIGN PATENTS

587,580 11/59 Canada.

DAVID L. RECK, Primary Examiner.

RAY K. WINDHAM, WINSTON A. DOUGLAS,  
Examiners.

UNITED STATES PATENT OFFICE  
CERTIFICATE OF CORRECTION

Patent No. 3,184,305

May 18, 1965

Sidney W. Poole et al.

It is hereby certified that error appears in the above numbered patent requiring correction and that the said Letters Patent should read as corrected below.

Columns 3 and 4, Table III, first column, line 5 thereof, for "4 Al-3 Mn" read -- 4 Al-4 Mn --; columns 5 and 6, Table V, third column, second section of the table, line 3 thereof, for "201.6" read -- 201.4 --; same section of Table V, seventh column, line 1 thereof, for "1757° F." read -- 1575° F. --; same columns 5 and 6, and columns 7 and 8, Table VI, for the column heading "Y.S. (k.s.i.), 2% offset", each occurrence, read -- Y.S. (k.s.i.), .2% offset --; column 8, line 33, for "iindicates" read -- indicates --; columns 9 and 10, Table VIII for the column heading "Y.S. (k.s.i.), 0.2% offset" read -- Y.S. (k.s.i.), .2% offset --; column 10, line 25, for "about" read -- above --; columns 11 and 12, Table IX, for the column heading "Y.S. (k.s.i.), 0.2+ offset" read -- Y.S. (k.s.i.), .2% offset --; same Table IX, fourth column, line 5 thereof, for "184.3" read -- 184.4 --; column 11, line 75, for "5/8 bar stock" read -- 5/8" bar stock --; column 14, line 13, before "silicon" insert -- zirconium, 0.1-0.5% by weight --; line 45, for "Crossley" read -- Crossley et al. --.

Signed and sealed this 30th day of November 1965.

(SEAL)  
Attest:

ERNEST W. SWIDER  
Attesting Officer

EDWARD J. BRENNER  
Commissioner of Patents